

June 20, 1933.

W. ROHN

1,915,243

METHOD OF PRODUCING CHROMIUM

Filed April 9, 1932

3 Sheets-Sheet 1

*Fig. 1.*



*Fig. 2.*



INVENTOR  
WILHELM ROHN  
BY *Stein & Rander*  
ATTORNEY

June 20, 1933.

W. ROHN

1,915,243

METHOD OF PRODUCING CHROMIUM

Filed April 9, 1932

3 Sheets-Sheet 2



INVENTOR  
WILHELM ROHN  
BY *W. Rohn*  
ATTORNEY

June 20, 1933.

W. ROHN

1,915,243

METHOD OF PRODUCING CHROMIUM

Filed April 9, 1932

3 Sheets-Sheet 3



INVENTOR  
WILHELM ROHN  
BY *Adolf Hauber*  
ATTORNEY

## UNITED STATES PATENT OFFICE

WILHELM ROHN, OF HANAU-ON-THE-MAIN, GERMANY, ASSIGNOR TO HERAEUS-VACUUMSCHMELZE A. G., OF HANAU-ON-THE-MAIN, GERMANY, A GERMAN COMPANY

## METHOD OF PRODUCING CHROMIUM

Application filed April 9, 1932, Serial No. 604,314, and in Germany April 15, 1931.

This invention relates to the art of metallurgy and more particularly to the production of chromium metal by the reduction of chromium oxide or ore by hydrogen.

5 Heretofore in the art it has been proposed to produce pure chromium by direct reduction of chromium oxide by hydrogen.

One process contemplates the reduction of chromium oxide in an externally heated tube 10 through which hydrogen is passed; but this cannot be carried on at a temperature higher than about 1560° C. because this is the highest temperature which the tube will withstand and at which it remains gas-tight. For 15 this method of operation the tubes must be of quite small diameter, and consequently the rate of production would be very limited. The main drawback to this method, however, is that hydrogen will not reduce 20 chromium oxide appreciably at 1560° C. unless it contains as little water-vapor as can be secured only by cooling the hydrogen to liquid air temperature. For these reasons 25 this procedure is not economically feasible for the production of chromium.

One of the objects of the present invention is to provide an improved method of reducing chromium oxides to chromium metal.

30 Another object is to provide apparatus for the reduction of chromium oxide to chromium metal.

Other objects and advantages will be apparent as the invention is further disclosed.

35 In accordance with the objects of the present invention I have found that when the source of heat is arranged within a containing vessel in such a way that the vessel itself remains cool, one may readily make

40 use of higher temperatures, up to and beyond about 1750° C. the melting point of chromium and even beyond 2000° C. This increase of temperature is, I have found, highly advantageous in that chromium oxide

45 at about 1700° C. is reduced by hydrogen dried by cooling it in the range -60° to -70° C., a range readily attained by the vaporization of a mixture of solid CO<sub>2</sub> with acetone, ether, trichlorethylene, etc., or of

50 ammonia under reduced pressure; and the

cost of thus freeing hydrogen to this extent from water vapor is only 1/10 to 1/15 of the cost when cooling to liquid air temperature is requisite. It is understood that another method of drying the hydrogen as by 55 absorption by P<sub>2</sub>O<sub>5</sub> or other drying agents is entirely equivalent to the freezing process described. A further economic advantage is that with internal heating a containing vessel of any size may be used so that large 60 charges of the oxide may thus be reduced in an atmosphere of hydrogen.

For this purpose one may use a heating element of molybdenum which enables temperatures of 2000° C. to be attained and is 65 perfectly stable in the atmosphere required for the reduction of the chromium oxide.

The necessary temperature can be still more advantageously reached and maintained by inductive heating of metallic 70 chromium, a small quantity of which is placed initially in the reaction chamber for this purpose. The chromium oxide is placed on this chromium, the vessel is closed and the requisite hydrogen atmosphere is established within it, and the current is turned on; the metal melts, reduction of the oxide begins, and the additional liquid metal so produced aids in the maintenance of the requisite high temperature by providing an 75 increasing amount of metal to be heated inductively. Or alternatively one may proceed by melting the initial amount of chromium inductively, placing on it the oxide to be reduced, closing the vessel and establishing the hydrogen atmosphere, with the same result; or one may proceed in any sequence of the several necessary steps.

Apparatus suitable for the purposes of the present invention is described in conjunction with the accompanying drawings wherein:—

Fig. 1 is a sectional side elevation view of a preferred type of induction heating furnace useful in the present invention;

Fig. 2 is a cross-sectional plan view of the same along plane 2—2 of Fig. 1;

Fig. 3 is a second sectional side elevation view of the same taken along plane 3—3 of Fig. 1;

Fig. 4 is a second cross-sectional plan view taken along plane 4—4 of Fig. 3;

Fig. 5 is a reduced sectional side elevation view of the same similar to Fig. 3 showing the associated reducing gas circulation and purifying apparatus schematically;

Fig. 6 is a sectional side elevation view of a modified furnace structure;

Fig. 7 is a cross-sectional view of the same; and

Fig. 8 is a sectional side elevation view of a second modified furnace structure.

Referring to the drawings, the preferred apparatus illustrates a furnace of the induction type which is specifically described and claimed in my copending application Serial No. 557,234 filed August 15, 1931. In this special type of furnace a low frequency current may be employed and the induced eddy currents produced by reason of the special coil design illustrated effects a stirring of the molten metal bath within the furnace from the bottom to the top thereby promoting and accelerating the rate of reduction of the chromium oxide on the top of the bath as well as facilitating and accelerating the rate of absorption of the reduced metal within the molten bath.

The furnace structure disclosed by the drawings substantially includes a crucible 1 interiorly faced with refractory material and a top 2 interiorly faced with refractory material and hermetically sealing the crucible 1 as indicated at 11, the hermetic seal being water cooled as indicated at 10. About the outer periphery of the crucible 1 are disposed a plurality of flat wound bowl shaped coils 3 substantially as indicated to conform with the contour of the peripheral face of the crucible as is more fully disclosed and claimed in my said above identified copending application. A core 5 is supported by pin 12 in a rotatable bearing carried by a support 4 at opposite sides of the crucible 1, the pin 12 in support 4 also serving to rotatably carry the entire weight of the crucible 1, top 2, coils 3 and core 5.

Crucible 1 is provided with two discharge openings as indicated in Figs. 3 and 4 each of which are normally closed by refractory elements 13 either of which are arranged to be readily removed when desired. Through the top 2 a gas inlet pipe 8 is provided and through one of the discharge openings a gas outlet pipe 9 is provided. In the normal operation of the furnace a head of pressure is maintained on the gas inflow such that the space enclosed within the crucible 1 and top 2 is substantially filled with gas at all times.

In accordance with the hereinabove described method I may place initially a small quantity of chromium metal 6 in the bottom of the crucible 1 and on the top thereof place the chromium oxide 7 which it is desired to reduce. The chromium oxide reduced

by the hydrogen during a reduction run incorporates with the chromium metal originally added and gradually builds up a larger molten bath of metal within the crucible 1.

The combined apparatus of the present invention is more clearly illustrated in Fig. 5 wherein is shown the induction furnace of Figs. 1 to 4 inclusive cooperatively connected with the reducing gas circulating and regenerating system. The elements heretofore identified with respect to the furnace structure and assembly are identified by similar numerals.

In Fig. 5 hydrogen of commercial purity is delivered to storage tank 40 through valve 79 wherein it is stored under pressure. From tank 40 it passes through valves 75 and 76 and appropriate piping into chamber 20 wherein it passes over cooling coils 22 carrying fluids or gases cooled to temperatures approximating  $-60^{\circ}$  to  $-70^{\circ}$  C. as hereinbefore described. Baffle plates 30 insure circulation of the hydrogen over coils 22. The thus purified hydrogen then passes through valves 77 and 78 and appropriate piping to inlet pipe 8 directly into the furnace wherein it circulates over the chromium oxide 7 which has been heated by conduction and radiation from molten bath 6 to temperatures at least approximating  $1700^{\circ}$  C. 15

The hydrogen is expelled from the furnace through pipe 9 in a strong free flow and passes directly into a second cooling and purifying chamber 20 which may be substantially identical with the first chamber 20 wherein it is circulated similarly over cooling coils 22 and thence returned through valves 71 and 72 and appropriate piping to pressure pump 34 operated by motor 36 which pump forces the substantially purified gas back into storage tank 40 through valves 73 and 74 and appropriate piping. 100

Cooling coils 22 in each purifying chamber 20 may be connected in series or in parallel as shown to refrigerating means 26 and a pump 24 should be provided to maintain circulation of the cooling fluid or gases therethrough. Chambers 20 should also be provided with suitable drain out means 28 substantially as indicated when coils 22 are defrosted. 110

Instead of using the type of furnace indicated in Figs. 1 to 4 inclusive, I may employ the type shown in Figs. 6 and 7, wherein a high frequency induction coil 108 with terminals 109 and 110 is used as a heating means. In such a furnace, container 100 preferably should be comprised of tubular or cylindrical non-metallic material such as glass quartz, glazed porcelain and the like. Crucible 102 may be of the shape illustrated or may be made more bowl shaped and also should be comprised of highly refractory materials non-reactive with chromium metal 106. Chromium oxide 104 is superposed upon the 120

metal 106 substantially as indicated and gas inlet means 8 and gas outlet means 9 are provided substantially as hereinbefore disclosed.

In this type of furnace, the solid piece of 5 chromium metal 106 is first incandesced and melted by high frequency induction heating by coil 108 and the chromium oxide 104 is progressively reduced by the circulating free flow of hydrogen thereover substantially as 10 hereinbefore described.

Referring to Fig. 8 a second modification 15 of furnace structure suitable for the purposes of the present invention contemplates the use of an incandescent heating element 120 instead of induction heating. By this means the reducing gas itself is heated to the requisite reducing temperature and thereby by radiation and conduction the metal oxide 104 retained in refractory crucible 102. Heating element 120 may be comprised of molybdenum as hereinbefore described and may be mounted substantially as shown with terminals 122 and 124 extending through the 20 wall of container 100. Other methods of 25 mounting heater 120 may be devised if desired.

Whereas the present invention has been described with particularity in connection with the use of substantially pure (moisture free) 30 hydrogen as a reducing agent it is not to be considered as being limited thereto. I have found that the reduction of the metal oxide may be effected also by substantially pure (moisture free) hydrogen in which there has 35 been incorporated a proportion of carbon-carrying gases such as hydrocarbon vapors, or even by admixtures of coke oven gases, water gas and other such fuel gases in accordance with the invention disclosed and claimed in 40 copending application Serial No. 642,464 filed November 12, 1932. The effect of the carbon is to accelerate the rate of reduction but the amount of such carbon that is introduced in the gas must be so controlled that 45 the resulting chromium is substantially free from carbon. It is to be understood that the present process involves the use of hydrogen substantially pure and free from moisture, but not necessarily excluding carbon-carrying 50 gases in such a limited proportion as will not permit the absorption of carbon by the metal.

The chromium produced in this way excels in purity other grades of chromium 55 hitherto manufactured commercially; for instance the chromium metal, as now prepared by the Goldschmidt process, contains varying amounts of aluminum and is otherwise not of constant composition.

Having broadly and specifically disclosed 60 the present invention it is apparent that many modifications and adaptations may be made therein without departing essentially from the nature and scope thereof as may be set forth in the following claims.

What I claim is:

1. The method of reducing chromium oxide with hydrogen which comprises heating the oxide to temperatures in excess of about 1600° C. and passing thereover a strong 70 free flow of hydrogen previously purified by exposure to temperatures ranging from about -60° C. to about -70° C.

2. The method of reducing chromium oxide with hydrogen which comprises subjecting the oxide to the action of a strong 75 free flow of hydrogen heated to temperatures in excess of about 1600° C., said hydrogen having been previously purified by exposure to temperatures ranging from 80 about -60° C. to about -70° C.

3. The method of producing substantially 85 pure chromium which comprises superposing chromium oxide upon a molten metal bath comprised substantially of pure chromium, and circulating thereover a strong free flow of substantially pure hydrogen having a water vapor content substantially not in excess of that retained therein subsequent to exposure to temperatures approximating -60° 90 C. to -70° C.

4. The method of producing substantially 95 pure chromium which comprises forming a molten metal bath comprised of substantially pure chromium, superposing thereon a quantity of chromium oxide and circulating thereover a strong free flow of substantially pure hydrogen, said hydrogen having a water vapor content substantially equivalent to that obtainable by exposure of the gas to temperatures approximating -60° C. to -70° C. 100

5. The method of reducing chromium oxide which comprises maintaining the chromium oxide at a temperature in excess of about 1750° C. and circulating thereover substantially pure hydrogen, said hydrogen having a water vapor content substantially equivalent to that obtained by cooling the gas to 105 temperatures between -60° C. and -70° C.

6. The method of producing substantially 110 pure chromium which comprises forming a molten metal bath comprised of substantially pure chromium, superposing thereon a quantity of chromium oxide, circulating thereover a strong free flow of substantially pure hydrogen having a water vapor content approximating that obtainable by exposure of the gas to temperatures approximating -60° C. to -70° C., and vigorously stirring the molten metal bath to facilitate the reduction 115 of the said oxide by the said hydrogen and the incorporation of the resultant metal product in the said bath.

7. The method of producing substantially 120 pure chromium which comprises forming a molten metal bath comprised of substantially pure chromium, superposing thereon a quantity of chromium oxide, vigorously stirring said bath by induced electric eddy currents and circulating thereover a strong free flow 125

of substantially pure hydrogen, said hydrogen having a water vapor content substantially equivalent to that obtainable by the exposure of the gas to temperatures approximating  $-60^{\circ}$  C. to  $-70^{\circ}$  C.

In witness whereof, I have hereunto signed my name.

WILHELM ROHN.

10

15

20

25

30

35

40

45

50

55

60

65